

July 7, 1936.

E. W. ISOM

2,046,749

MANUFACTURE OF MOTOR FUEL

Filed May 1, 1930



INVENTOR

Edward W. Isom

BY

Pearce, Davis, Marvin & Edwards

ATTORNEYS

## UNITED STATES PATENT OFFICE

2,046,749

## MANUFACTURE OF MOTOR FUEL

Edward W. Isom, Scarsdale, N. Y., assignor to  
 Sinclair Refining Company, New York, N. Y., a  
 corporation of Maine

Application May 1, 1930, Serial No. 448,929

3 Claims. (Cl. 196—58)

This invention relates to improvements in the manufacture of motor fuel gasoline. The invention has several advantages and includes improvements important in several respects.

5 The invention provides for the production of motor fuel gasoline and dry, merchantable coke, or motor fuel gasoline, distillates of gas oil of kerosene character and dry, merchantable coke, as end products, without involving the production of residual fuel oil or low grade coke.

10 The invention is applicable generally to a wide range of stocks, including clean stocks and dirty stocks. It is applicable, for example, to kerosene, gas oil, relatively clean reduced crude oil, 15 relatively dirty reduced crude oil, residual fuel oil including residuals produced in cracking operations, tars, etc.

15 In one aspect, the invention provides for the conversion of residual fuel oil, produced in other operations, into more valuable products, motor fuel gasoline and dry, merchantable coke or motor fuel gasoline, distillates of gas oil of kerosene character and dry, merchantable coke.

20 The invention provides for an increase in the recovery of motor fuel gasoline, or motor fuel gasoline and distillates of gas oil of kerosene character, from higher boiling stocks, and particularly from dirty higher boiling stocks.

25 The invention provides for the production of motor fuel gasoline by severe cracking operations producing anti-knock values of a high order but improved with respect to stability.

30 The several advantages of the invention are, moreover, secured in an operation of satisfactory economy.

35 In one aspect, the invention includes improvements in the processes described in Letters Patent No. 1,757,843 issued to Sinclair Refining Company, May 6, 1930, on an application of Eugene C. Herthel and Harry L. Peizer and in application Serial No. 340,996, filed February 18, 1929, by Harry L. Peizer.

40 The invention comprises the maintenance of free hydrogen in an extreme state of dispersion in a high temperature region of active reaction through which the hot oil products of a severe cracking operation pass while still at high temperature and through which pitch constituents pass as they are about to become coke. The free hydrogen may be introduced as such, or it may be produced, or in part produced, within the region of reaction by the introduction of steam, under appropriate conditions.

45 The temperature of the region of reaction may be maintained by the heat of the hot oil products

of the severe cracking operation passing therethrough. Additional heat may be supplied by superheating the hydrogen or hydrogen-containing gas, or steam, introduced into the region of reaction.

5 The pressure in the region of reaction may vary from a pressure approximating atmospheric pressure up to a pressure of several hundred pounds per square inch, for example, or more. However, one important advantage of the invention is that it does not necessitate the maintenance of high pressures but may be carried out under relatively low pressure.

10 In carrying out the invention, hot oil products from a severe cracking operation, the superheated hydrocarbon vapors and gases from a vapor-phase cracking operation, for example, are passed through a liquid body of oil, being introduced into the liquid body of oil beneath its liquid level and passed upwardly therethrough, the oil thus being reduced to coke, and free hydrogen, or a gas mixture rich in free hydrogen, is passed through the liquid body of oil together with the hot oil products from the severe cracking operation. Steam may be passed through the liquid body in 15 addition to the hydrogen or hydrogen-containing gas, or under appropriate conditions, steam may be passed through the liquid body of oil, and coke, with the hot oil products from the severe cracking operation instead of the hydrogen 20 or hydrogen-containing gas.

25 The coking operation is carried out as described in Letters Patent No. 1,757,843, mentioned above. In the coking operation, the initial formation of coke establishes a dispersion 30 means about the point of introduction of the hot oil products from the severe cracking operation peculiarly effective in accomplishing dispersion to an extreme degree of the superheated gases and vapors entering the overlying oil and 35 pitch, through the coke formed. As pitch is formed in the oil body, in excess of that soluble in the oil, it precipitates as a film overlying the accumulating coke and undergoing conversion to coke.

40 Following the initial formation of coke, gas introduced through the coke is similarly subject to extreme dispersion in the oil and pitch overlying the accumulating coke, whether introduced at the point of introduction of the hot oil products from the severe cracking operation or, into the coke, at some other point.

45 The region including the film of pitch overlying the accumulating coke and the adjacent coke and oil is the "region of active reaction" 50

55

to which reference has been made. Within this region, the oil and pitch constituents present are, at the prevailing high temperature, normally reactive and the gases and vapors passing through this region are, at the prevailing high temperature and because of the extreme dispersion to which they are subjected, super-normally reactive.

In one aspect, the super-normally reactive condition of the vapors and gases within the region of reaction effected by extreme dispersion of the vapors and gases in carrying out the invention, makes it possible to maintain satisfactory reaction rates under relatively low pressures; in another aspect, it makes it possible to maintain high reaction rates under high pressures.

Where the accumulating coke is maintained at a temperature upwards of 1200° F. or thereabout, steam may be introduced into the region of reaction, instead of hydrogen or a hydrogen-containing gas. Within the temperature range of the "water gas reaction", steam introduced into the region of reaction will react with the coke to form free hydrogen and carbon monoxide, hydrogen so formed being introduced into the region of reaction in a nascent state.

While the invention involves the production of coke as an end product, the coke produced is a valuable, dry, merchantable coke and the proportion of coke produced with respect to the oil treated is small and may be made very small.

In the region of reaction, the more reactive constituents of the motor fuel gasoline component of the hot oil products discharged from the severe cracking operation, producing instability in the motor fuel product, are subjected to conditions converting such constituents into less reactive and more stable constituents of the motor fuel product or of the gas oil of kerosene character distillate products and into pitch in turn converted into coke. Because of the high temperature prevailing in the region of reaction, the resulting motor fuel gasoline product, although of improved stability, retains in large measure the anti-knock values produced in the severe cracking operation. The motor fuel gasoline product of the invention is thus to be distinguished from gasoline products produced, for example, by simple "hydrogenation" of a gasoline produced by a severe cracking operation.

The invention will be further described in connection with the accompanying drawing, which illustrates, diagrammatically and conventionally, in elevation and partly in section and with parts broken away, one form of apparatus adapted for carrying out the invention. It will be understood that the invention may be carried out in other and in different forms of apparatus; the particular apparatus illustrated in the accompanying drawing is illustrated merely for purposes of exemplification.

The apparatus illustrated comprises a coking receptacle 1, within which the "region of active reaction" of the invention is maintained during operation, a cracking heater 2, a superheater 3, a scrubbing tower 4, fractionating towers 5 and 6, a condenser 7 and a receiver 8. The cracking heater 2 and the superheater 3 are arranged to discharge into the lower end of the coking receptacle 1 through connection 9. Vapors and gases escaping from the upper part of the coking receptacle 1 are discharged, in normal operation, into and beneath the liquid level of a liquid body of oil maintained in the lower end of

the scrubbing tower 4 through connections 10 and 11. The oil mixture constituting the liquid body maintained in the lower part of the scrubbing tower 4 is forced into the upper part of the coking receptacle 1 through connections 12 and 13 by means of pump 14. Vapors and gases escaping from the upper part of the scrubbing tower 4 are discharged into the lower part of the fractionating tower 5 through connection 15. The oil mixture collecting in the lower part of the fractionating tower 5 is supplied to the cracking heater 2 through connections 16 and 17 by means of pump 18. Vapors and gases escaping from the upper part of the fractionating tower 5 are discharged either into the lower part of the fractionating tower 6 through connections 19 and 20, or directly to the condenser 7 through connections 19, 21 and 22. Vapors and gases escaping from the upper part of fractionating tower 6 are discharged to the condenser 7 through connection 22. Condensate is discharged from the receiver 8 through connection 23, uncondensed vapors and gases being discharged therefrom through connection 24. Each of the towers 4, 5 and 6 is illustrated as provided for purposes of control, with a reflux condenser 25, 26 and 27 respectively. A condenser 28 and steam connection 29 are provided for steaming out the coking receptacle 1 at the end of a run. Connection 30 is provided for supplying steam to the lower part of the scrubbing tower 4.

A vapor-phase cracking operation, for example, may be carried out in the cracking heater 2. A gas oil or kerosene character stock or stock mixture, for example, may be supplied through connection 17 and heated to a temperature, as discharged through connection 31, approximating 1100-1200° F. under a pressure, as discharged through connection 31, approximating 10-20 pounds per square inch (above atmospheric pressure). Such a vapor-phase cracking operation may be carried out, for example, as described in application, Serial No. 198,621, filed June 13, 1927, by Harry L. Pelzer, and the hot oil products therefrom, discharged through connections 31 and 9, or the digesting drums may be omitted, as in the apparatus illustrated in the accompanying drawing. Or a gas oil or kerosene character stock or stock mixture, for example, may be heated to a temperature, as discharged through connection 31, approximating 1000-1150° F. under a pressure, as discharged through connection 31, as high as 400-600 pounds per square inch or higher.

The scrubbing tower 4 and the fractionating towers 5 and 6 may be operated, for example, as described in application Serial No. 345,199, filed March 7, 1929, by Eugene C. Hertel. A liquid body of oil, from which liquid oil is supplied to the coking receptacle and to which raw oil and entrained constituents scrubbed from the vapors and gases escaping from the coking receptacle are supplied, is maintained in the lower part of the scrubbing tower 4 and the vapors and gases escaping from the coking receptacle 1 are discharged into and beneath the liquid level of this liquid body of oil through connection 11. Raw oil, particularly relatively dirty raw oil, reduced crude oil for example, may be supplied to the scrubbing tower 4 at an intermediate point, through connection 32, or better, directly to the liquid body of oil in the lower part of the scrubbing tower 4, through connection 33. Raw oil, particularly relatively clean raw oil, a gas oil or

kerosene character stock for example, may be supplied to the upper part of the scrubbing tower 4 as a refluxing medium, through connection 34. The operation of the scrubbing tower 5 may be controlled, or control effected by raw oil supplied through connection 32 or connection 34 or both of these connections may be supplemented by regulated circulation of a cooling medium through the reflux condenser 25. Where both of the fractionating towers 5 and 6 are used, a relatively higher boiling fraction is separated in the tower 5 and a relatively lower boiling fraction in the tower 6. Either or both of these fractions, together with any admixed raw oil introduced into the fractionating towers 5 or 6 or either of them, may be supplied to the cracking heater 2. The operation of the fractionating towers 5 and 6 may be controlled by the regulated introduction of raw oil, best 10 relatively clean raw oil, a gas oil or kerosene character stock for example, through connections 35 and 36 or by regulated circulation of a cooling medium through the reflux condensers 26 and 27, or by both of these means conjointly. 15 The vapors and gases escaping to the condenser 7 through connection 22 may be subjected to direct refining treatment on their way to the condenser. For example, this gas-vapor mixture may be subjected to direct refining treatment 20 as described in application Serial No. 257,958, filed February 29, 1928, by Eugene C. Herthel.

The coking receptacle 1 is, with advantage, arranged and operated with respect to the scrubbing tower 4 as described in application Serial No. 340,996, filed February 18, 1929, by Harry L. Pelzer. The coking receptacle 1 may, with advantage, be arranged as described in application, Serial No. 344,952, filed March 7, 1929, by Oliver F. Campbell and Eugene C. Herthel for the purpose of discharging accumulated charges of coke. Since individual coking receptacles must be operated intermittently to permit the discharge of accumulated charges of coke, a plurality of coking receptacles may be provided to 40 permit the general operation to be carried out continuously. Such a group of coking receptacles may, with advantage, be operated as described in application Serial No. 341,214, filed February 19, 1929, by Harry L. Pelzer.

In carrying out the invention in the apparatus illustrated, the gas and vapor mixture introduced into the lower end of the coking receptacle 1 through connection 9 includes, in addition to the hot oil products discharged from the cracking heater 2, hydrogen or a hydrogen-containing gas or steam or a mixture of two or more of these gases supplied either through connection 37 or through connection 38 or through both of these connections. Suitable gas mixtures include mixtures of hydrogen and hydrocarbon gases, produced, for example, by thermal decomposition of hydrocarbon gas mixtures. The gas mixture escaping through connection 24, for example, including any remaining free hydrogen, may be reintroduced into the lower end of the coking receptacle 1 through connection 9 and the free hydrogen content of the reintroduced gases may first be increased by the addition of free hydrogen or by the subjection of the gas mixture to thermal decomposition. Such thermal decomposition of hydrocarbon gases may be effected, for example, by passing the gases through checker-work or coke maintained at a temperature upwards of 1200-1400° F. The hydrogen or hydrocarbon-containing gas or steam introduced into the

lower end of the coking receptacle 1 is superheated, if necessary, to a temperature sufficient to maintain the requisite temperature within the region of reaction in the coking receptacle. The apparatus illustrated includes a superheating 5 furnace 3 for this purpose. Steam may be superheated in the heating coil 39 and hydrogen or a hydrogen-containing gas may be superheated in the heating coil 40. It will be understood that a separate super-heating furnace may be provided 10 for superheating steam and the hydrogen or hydrogen-containing gas separately or that only the steam or only the hydrogen or hydrogen-containing gas may be superheated.

In carrying out the invention in the apparatus illustrated, a mixture of the hot oil products discharged from the cracking furnace 2 and hydrogen or hydrogen-containing gas is introduced into the lower end of the coking receptacle 1, at a temperature as introduced approximating 1150- 1300° F. for example, through a body of coke, formed about the inlet from the connection 9 as the operation of the coking receptacle is initiated, into a fluid body of oil and pitch overlying the accumulating coke and from which pitch is precipitating upon the accumulating coke, undergoing as precipitated conversion to coke. As the introduced mixture of vapors and gases passes through the accumulating coke, it is subdivided 25 to enter the overlying oil and pitch dispersed to 30 an extreme degree therethrough. This extreme dispersion enormously increases the area of contact between the vapors and gases and the oil and pitch, particularly within the region immediately adjacent to the upper level of the 35 accumulating coke, thus promoting heat transfer between the vapors and gases and the oil and pitch and affording the maximum opportunity for the attainment of the equilibrium represented by the concentration of free hydrogen within this 40 region. The concentration of free hydrogen with respect to the oil and pitch within this region may be increased by increasing the pressure prevailing in the coking receptacle. The coking receptacle 1 may be operated, for example, under 45 a pressure approximating 0-10 pounds per square inch or under a pressure approximating 90-150 pounds per square inch or under a pressure approximating 300-350 pounds per square inch or under higher pressures. The temperature of the 50 vapors and gases escaping from the upper part of the coking receptacle 1 may be maintained, for example, in the neighborhood of 1050-1250° F. and may advantageously be increased somewhat as coke accumulates within the coking receptacle.

The invention will be further exemplified by the following examples of operations embodying the invention as carried out in the apparatus 55 illustrated:

An oil mixture comprising reduced crude oil, having a gravity of about 15 A. P. I., is supplied to the coking receptacle 1 through connection 13 at a rate of about 250-450 gallons per hour and at a temperature approximating 750-800° F. A 60 gas oil character stock, having a gravity of about 35 A. P. I., is supplied to the cracking heater 2 through connection 17 at a rate of about 900-1200 gallons per hour and heated therein to a 65 temperature, as discharged through connection 31, approximating 1160-1180° F. under a pressure, as discharged through connection 31, approximating 20 pounds per square inch. Free hydrogen preheated to a temperature sufficient to bring 70 75

- the temperature of the resulting mixture passing through connection 9 to about 1200-1250° F. is supplied through connection 38 at a rate of about 30,000-60,000 cubic feet (under standard conditions) per hour. The coking receptacle 1 is maintained under a pressure approximating 3-5 pounds per square inch.
- An oil mixture comprising residual tar from pressure distillation cracking operations, having a gravity of about 20 A. P. I., is supplied to the coking receptacle 1 through connection 13 at a rate of about 350-500 gallons per hour and at a temperature approximating 750-800° F. A gas oil character stock, having a gravity of about 35 A. P. I., is supplied to the cracking heater 2 through connection 17 at a rate of about 1000-1500 gallons per hour and heated therein to a temperature, as discharged through connection 31, approximating 1160-1180° F. under a pressure, as discharged through connection 31, approximating 20 pounds per square inch. A hydrocarbon gas mixture including about 35% free hydrogen preheated to a temperature sufficient to bring the temperature of the resulting mixture passing through connection 9 to about 1200-1300° F., is supplied through connection 38 at a rate of about 50,000-100,000 cubic feet per hour. The coking receptacle 1 is maintained under a pressure approximating 3-5 pounds per square inch.
- An oil mixture comprising reduced crude oil, having a gravity of about 15 A. P. I., is supplied to the coking receptacle 1 through connection 13 at a rate of about 200-300 gallons per hour and at a temperature approximating 750-800° F. A kerosene character stock, having a gravity of about 40 A. P. I., is supplied to the cracking heater 2 through connection 17 at a rate of about 1000-1200 gallons per hour and heated therein to a temperature, as discharged through connection 31, approximating 1175-1200° F. under a pressure, as discharged through connection 31, approximating 200-250 pounds per square inch. Free hydrogen preheated to a temperature sufficient to bring the temperature of the resulting mixture passing through connection 9 to about 1200-1300° F. is supplied through connection 38 at a rate of about 40,000-65,000 cubic feet per hour. The coking receptacle 1 is maintained under a pressure approximating 3-5 pounds per square inch.
- An oil mixture comprising reduced crude oil, having a gravity of about 15 A. P. I., is supplied to the coking receptacle 1 through connection 13 at a rate of about 200-300 gallons per hour and at a temperature approximating 750-800° F. A gas oil character stock having a gravity of about 35 A. P. I. is supplied to the cracking heater 2 through connection 17 at a rate of about 900-1200 gallons per hour and heated therein to a temperature, as discharged through connection 31, approximating 1050-1150° F. under a pressure, as discharged through connection 31, approximating 400 pounds per square inch. A hydrocarbon gas mixture including about 50% free hydrogen preheated to a temperature sufficient to bring the temperature of the resulting mixture passing through connection 9 to about 1200-1250° F. is supplied through connection 38 at a rate of about 40,000-80,000 cubic feet per hour. The coking receptacle 1 is maintained under a pressure approximating 100-125 pounds per square inch.
- An oil mixture comprising reduced crude oil, having a gravity of about 15 A. P. I., is supplied to the coking receptacle 1 through connection 13 at a rate of about 300-400 gallons per hour and

at a temperature approximating 750-800° F. A kerosene character stock, having a gravity of about 40 A. P. I., is supplied to the cracking heater 2 through connection 17 at a rate of about 1000-1200 gallons per hour and heated therein to a temperature, as discharged through connection 31, approximating 1175-1200° F. under a pressure, as discharged through connection 31, approximating 500-600 pounds per square inch. Free hydrogen preheated to a temperature sufficient to bring the temperature of the resulting mixture passing through connection 9 to about 1200-1300° F. is supplied through connection 38 at a rate of about 50,000-75,000 cubic feet per hour. The coking receptacle 1 is maintained under a pressure approximating 400-500 pounds per square inch.

An oil mixture comprising reduced crude oil, having a gravity of about 15 A. P. I. is supplied to the coking receptacle 1 through connection 13 at a rate of about 200-300 gallons per hour at a temperature approximating 750-800° F. A kerosene character stock, having a gravity of about 40 A. P. I., is supplied to the cracking heater 2 through connection 17 at a rate of about 900-1000 gallons per hour and heated therein to a temperature, as discharged through connection 31, approximating 1150-1200° F. under a pressure, as discharged through connection 31, approximating 20 pounds per square inch. A gas mixture including about 40% free hydrogen and 60% steam preheated to a temperature sufficient to bring the temperature of the resulting mixture passing through connection 9 to about 1200-1300° F. is supplied through connections 37 and 38 at a rate of about 20,000-50,000 cubic feet per hour. The coking receptacle 1 is maintained under a pressure approximating 3-5 pounds per square inch.

An oil mixture comprising reduced crude oil, having a gravity of about 15 A. P. I., is supplied to the coking receptacle 1 through connection 13 at a rate of about 300-500 gallons per hour and at a temperature approximating 750-800° F. A gas oil character stock, having a gravity of about 35 A. P. I., is supplied to the cracking heater 2 through connection 17 at a rate of about 1000-1500 gallons per hour and heated therein to a temperature, as discharged through connection 31, approximating 1160-1180° F. under a pressure, as discharged through connection 31, approximating 20 pounds per square inch. A gas mixture including about 30% of steam, 20% of free hydrogen and 50% of hydrocarbons preheated to a temperature sufficient to bring the temperature of the resulting mixture passing through connection 9 to about 1250-1300° F. is supplied through connections 37 and 38 at a rate of about 30,000-65,000 cubic feet per hour. The coking receptacle 1 is maintained under a pressure approximating 3-5 pounds per square inch.

An oil mixture comprising reduced crude oil, having a gravity of about 15 A. P. I., is supplied to the coking receptacle 1 through connection 13 at a rate of about 250-450 gallons per hour and at a temperature approximating 750-800° F. A gas oil character stock having a gravity of about 35 A. P. I. is supplied to the cracking heater 2 through connection 17 at a rate of about 900-1200 gallons per hour and heated therein to a temperature, as discharged through connection 31, approximating 1175-1200° F. under a pressure, as discharged through connection 31, approximating 20 pounds per square inch. Steam pre-

heated to a temperature sufficient to bring the temperature of the resulting mixture passing through connection 9 to about 1250-1300° F. is supplied through connection 37 at a rate of about 5 40,000-80,000 cubic feet per hour. The coking receptacle 1 is maintained under a pressure approximating 3-5 pounds per square inch.

An oil mixture comprising reduced crude oil, having a gravity of about 15 A. P. I., is supplied 10 to the coking receptacle 1 through connection 13 at a rate of about 200-300 gallons per hour and at a temperature approximating 750-800° F. A kerosene character stock having a gravity of about 40 A. P. I., is supplied to the cracking heater 2 through connection 17 at a rate of about 15 1000-1500 gallons per hour and heated therein to a temperature, as discharged through connection 31, approximating 1175-1200° F. under a pressure, as discharged through connection 31, 20 approximating 200-250 pounds per square inch. Steam preheated to a temperature sufficient to bring the temperature of the resulting mixture passing through connection 9 to about 1250-1300° F. is supplied through connection 38 at a rate of 25 about 50,000-75,000 cubic feet per hour. The coking receptacle 1 is maintained under a pressure approximating 150-200 pounds per square inch.

The gas mixtures containing free hydrogen 30 more particularly useful in carrying out the invention are those containing upwards of 20% or, better, upwards of 30% of free hydrogen. In referring to severe cracking operations, reference is intended to cracking operations in which 35 oil is heated to a temperature high enough, generally upward of 950° F., to produce a motor fuel gasoline product having anti-knock values of a high order.

I claim:

40 1. In the manufacture of motor fuel gasoline, the improvement which comprises subjecting an oil to severe vapor phase cracking conditions upwards of 950° F., thereby producing a mixture of vapors and gases, heating an additional gas mix-

ture containing upwards of about 20% of free hydrogen to a temperature upwards of 1200° F., simultaneously passing the highly heated vapors and gases from the vapor phase cracking operation together with the additional highly heated 5 hydrogen-containing gas mixture upwards through an accumulating body of coke into an overlying body of oil and pitch undergoing conversion to coke.

2. In the manufacture of motor fuel gasoline, 10 the improvement which comprises subjecting an oil to severe vapor phase cracking conditions upwards of 950° F., thereby producing a mixture of vapors and gases, heating an additional gas mixture containing upwards of about 20% of free 15 hydrogen to a temperature upwards of 1200° F., simultaneously passing the highly heated vapors and gases from the vapor phase cracking operation together with the additional highly heated hydrogen-containing gas mixture upwards 20 through an accumulating body of coke into an overlying body of oil and pitch undergoing conversion to coke at a temperature upwards of 1200° F.

3. In the manufacture of motor fuel gasoline, 25 the improvement which comprises subjecting an oil to severe vapor phase cracking conditions upwards of 950° F., thereby producing a mixture of vapors and gases, superheating steam to a 30 temperature substantially in excess of 1200° F., uniting the superheated steam and the vapors and gases from the vapor phase cracking operation, introducing the mixture at a temperature in excess of 1200° F. upwardly into a coking zone 35 adapted to receive an accumulating charge of coke, and passing the mixture of superheated steam and the hot products from the vapor phase cracking operation upwardly through a body of coke accumulating in said coking zone and into 40 an overlying body of oil and pitch undergoing conversion to coke at a temperature upwards of 1200° F.

EDWARD W. ISOM.